

June 8, 1948.

N. A. ZIEGLER

2,442,944

FERROUS ALLOY

Filed May 15, 1944

2 Sheets-Sheet 1

*Fig. 1.*



*Fig. 2.*



Forventor:  
Nicholas A. Ziegler  
By: Joseph O. Lange, Atty.

June 8, 1948.

N. A. ZIEGLER

2,442,944

FERROUS ALLOY

Filed May 15, 1944

2 Sheets-Sheet 2

*Fig. 3.*



*Fig. 4.*



Inventor:  
Nicholas A. Ziegler  
By: Joseph O. Lange, Atty.

## UNITED STATES PATENT OFFICE

2,442,944

## FERROUS ALLOY

Nicholas A. Ziegler, Chicago, Ill., assignor to  
 Crane Co., Chicago, Ill., a corporation of  
 Illinois

Application May 15, 1944, Serial No. 535,704

2 Claims. (CL 75—128)

1

This invention relates to ferrous alloys and more particularly to chromium-molybdenum steels with low carbon content.

Steels of this type are commonly used for the construction of pressure-containing vessels and parts, such as valve bodies, bonnets, discs and the like. Such structures are frequently fabricated and installed in service by welding and thus new problems arise with respect to the physical properties of the steel alloys employed. Not only must the cast members exhibit acceptable strength properties before fabrication, but the final assembly after fabrication must be structurally strong, free from porosity, internal strains, and capable of withstanding the stresses resulting from high operating pressures.

Previous investigations and studies of chromium-molybdenum steels in the range of 2.5-9% Cr, 0-2% Mo and 0-0.3% C have indicated that, generally speaking, a reduction in the carbon content will give better thermal properties, that is, less susceptibility to thermal cracks when the material cools down in the mold from the liquid state, as well as when it is subjected to various heat treating operations, involving rapid cooling, such as normalizing or quenching. Reduced susceptibility to thermal cracking is particularly important during welding, when rapid alternate heating and cooling is a part of the operation. It is therefore desirable to reduce the carbon content to as low a figure as possible without impairing the strength properties. It has been found that when the carbon content of these steels is decreased to values below 0.10%, the strength of the resultant steel decreases very rapidly. This decrease is serious in commercial steels which must meet the following requirements set up by various engineering bodies such as, for example, the American Society for Testing Materials:

One of the important objects of this invention is to provide a chromium-molybdenum steel of low carbon content and suitable as a material for the cast members of pressure vessels, such as valves or the like, the complete structures of which are fabricated by welding the individual cast members into an assembled unit.

Another object of this invention is the provision of an alloy steel of such favorable thermal properties and welding characteristics as to permit the fabrication of cast members into pressure-containing bodies characterized by freedom from porosity, internal strains and high resistance to stresses resulting from operating pressure.

A further object of this invention is the provision of a welding steel adapted to the construction of welded pressure vessels which will have the required tightness, strength and freedom from internal strains without the necessity of stress-relieving the welded portions.

With the foregoing objects in view, I have discovered that the addition of nickel in small amounts to low-carbon chromium-molybdenum steels of a definite compositional range will have a marked strengthening effect on the resulting physical properties, without making them unduly thermally sluggish, air hardenable, susceptible to internal strains, thermal cracks or difficult to weld. While the addition of nickel to steels of this type is known to have a beneficial effect upon the physical properties, no one, to my knowledge, has discovered the effect of the addition of definite amounts of nickel upon the welding qualities of chromium-molybdenum steels of low carbon content.

To investigate the effect of nickel on the welding qualities of this type of steel, some direct welding experiments were performed. Parts of 40 castings made of eight experimental steels were

| Minimum                              |                              |                         |                                   |                                   | Maximum<br>Brinell<br>Hardness<br>Number |
|--------------------------------------|------------------------------|-------------------------|-----------------------------------|-----------------------------------|------------------------------------------|
| Tensile<br>Strength,<br>lbs./sq. in. | Yield Point,<br>lbs./sq. in. | Elongation,<br>Per cent | Reduction<br>of Area,<br>Per cent | Impact<br>Resistance,<br>ft.-lbs. |                                          |
| 90,000                               | 65,000                       | 18                      | 30                                | 15                                | 235                                      |

sectioned and then arc-welded together in their original shapes, using chromium-molybdenum electrodes of the following specified composition:

|           | Percent  | 5  |
|-----------|----------|----|
| C (max.)  | 0.10     |    |
| Cr        | 4-6      |    |
| Mo        | 0.4-0.65 |    |
| Mn (max.) | 0.75     |    |
| Si (max.) | 0.75     |    |
| P (max.)  | 0.03     | 10 |
| S (max.)  | 0.03     |    |

The compositions of the eight experimental steels tested are shown in Table 1 below.

TABLE 1

| Serial No. | Composition |      |       |       |      |      |      |      |
|------------|-------------|------|-------|-------|------|------|------|------|
|            | Si          | Mn   | S     | P     | C    | Ni   | Cr   | Mo   |
| 1.         | 0.32        | 0.01 | 0.023 | 0.028 | 0.20 | 0.02 | 5.22 | 0.62 |
| 2.         | 0.31        | 0.69 | 0.022 | 0.030 | 0.24 | 1.16 | 5.34 | 0.64 |
| 3.         | 0.56        | 0.67 | 0.026 | 0.020 | 0.09 | 0    | 4.39 | 0.51 |
| 4.         | 0.77        | 0.69 | 0.021 | 0.022 | 0.09 | 1.30 | 4.68 | 0.48 |
| 5.         | 0.65        | 0.64 | 0.020 | 0.024 | 0.10 | 0.63 | 7.22 | 1.08 |
| 6.         | 0.56        | 0.60 | 0.026 | 0.028 | 0.10 | 1.17 | 7.11 | 1.10 |
| 7.         | 0.74        | 0.59 | 0.023 | 0.034 | 0.12 | 0.02 | 8.94 | 1.45 |
| 8.         | 0.61        | 0.59 | 0.023 | 0.030 | 0.07 | 1.29 | 9.01 | 1.78 |

It may be noted that the prime object of adding molybdenum to these types of steels is to develop a desired high temperature creep resistance.

Vickers hardness tester and taking readings at about  $\frac{1}{8}$  inch intervals across the weld and affected zone. (Vickers readings for these types of steels are directly comparable to Brinell numbers.) Figs. 1-4 of the drawings accompanying this specification are graphic representations of these hardness distribution studies, in which

Fig. 1 represents steels containing 5% Cr, 0.5% Mo and 0.2% C;

Fig. 2 represents steels containing 5% Cr, 0.5% Mo and 0.1% C;

Fig. 3 represents steels containing 7% Cr, 1% Mo and 0.1% C, and

Fig. 4 represents steels containing 9% Cr, approximately 2% Mo and 0.1% C.

Generally speaking, Fig. 1 represents high-carbon steels and Figs. 2, 3 and 4 represent low-carbon steels. In each case, the dotted-line curve represents a nickel-free steel and the solid-line curve represents a steel containing 1% nickel. The numbers along the vertical axes of these curves represent Vickers hardness units. The numbers 1-10 along the horizontal axes designate the location of the points in the various zones of the welded section at which Vickers hardness readings were taken.

In order to demonstrate that the steels treated according to this invention were improved in physical properties, the results of physical tests are presented in Table 2 below.

TABLE 2  
Tensile properties

| Serial No. | Tensile Strength, p. s. i. | Yield Point, p. s. i. | Proportional limit, p. s. i. | Elongation, Per Cent | Reduction of Area, Per Cent | Charpy Impact Resistance |              | Hard. B. H. N. |
|------------|----------------------------|-----------------------|------------------------------|----------------------|-----------------------------|--------------------------|--------------|----------------|
|            |                            |                       |                              |                      |                             | Ft. R. T.                | Lbs. -25° F. |                |
| 1.         | 106,000                    | 75,000                | 46,000                       | 23.5                 | 60.5                        | 23.0                     | 14.0         | 230            |
| 2.         | 101,000                    | 76,000                | 59,000                       | 24.0                 | 61.0                        | 19.0                     | 8.0          | 308            |
| 3.         | 80,000                     | 53,000                | 36,000                       | 32.0                 | 70.0                        | 31.0                     | 20.0         | 232            |
| 4.         | 101,000                    | 75,000                | 64,000                       | 23.0                 | 65.0                        | 27.0                     | 9.0          | 206            |
| 5.         | 76,000                     | 52,000                | 37,000                       | 32.5                 | 67.5                        | 26.5                     | 24.5         | 215            |
| 6.         | 101,000                    | 78,000                | 66,000                       | 22.0                 | 64.0                        | 26.0                     | 17.0         | 202            |
| 7.         | 88,000                     | 68,000                | 47,000                       | 23.0                 | 63.5                        | 25.0                     | 13.5         | 232            |
| 8.         | 110,000                    | 71,000                | 56,000                       | 22.0                 | 64.0                        | 35.0                     | 22.0         | 230            |

(The analyses of these steels are given in Table 1.)

ance. When the amount of chromium exceeds about 2 per cent, molybdenum in amounts up to about 2 per cent has relatively small effect on the room temperature physical properties and thermal characteristics.

While the experimental data presented relate specifically to compositions including chromium contents up to about 9%, I have found that the favorable results to be gained by the practice of this invention will apply to steels of this type containing chromium contents of up to 12%, since this represents the known upper limit of chromium for heat treatability with low carbon. The eight experimental steels were heat treated by (1) normalizing from 1750° F., (2) air quenching from 1550° F. and (3) drawing at 1250-1300° F.

In summary, the range of analysis (in percent) of my improved weldable cast steel is chromium from 2 to 10%, molybdenum .5 to 2%, with the usual amounts of silicon, manganese, sulphur and phosphorus, nickel from .75 to 1.5%, preferably not over .10% carbon and with the balance iron and incidental impurities.

A transverse section was cut from each of the welds (without stress-relieving them) and the sections roughly polished. A hardness survey was made over each of these test pieces using a

Referring now to Tables 1 and 2, it may be noted that steels 1 and 2 are standard 4-6% Cr, 0.5% Mo steels containing 0.2% C. No. 1 contains no nickel and No. 2 contains 1.0% nickel. Both meet the A. S. T. M. specifications given above, except that No. 2 is slightly hard. All the rest of the steels contain 0.1% C, i. e. half of the carbon contents of Nos. 1 and 2. Nos. 3 and 4 contain 4-6% Cr, 0.5% Mo; Nos. 5 and 6 contain 7% Cr and 1% Mo, and Nos. 7 and 8 contain 9% Cr and 1.5% Mo. In each of these three pairs the first steel is nickel-free or low in nickel and the second contains 1% Ni. The point of interest is the fact that the tensile strength of the three nickel-free steels is below 90,000 pounds per square inch (A. S. T. M. specification) and the tensile strength of the three nickel-bearing steels is about 100,000 pounds per square inch. Likewise, the yield point of two of the three nickel-free steels is below the A. S. T. M. specification of 65,000 pounds per square inch and the yield point of the three nickel-bearing steels is above 70,000 pounds per square inch. At the same time, the elongation, reduction of area and impact resistance, at room temperature, of all these steels are well above 18%, 30% and 15 foot-pounds, respectively, that is, the A. S. T. M. specifications. Likewise, the hardness of

all these steels is below the A. S. T. M. maximum of 235. Thus, the addition of nickel in amounts of about 1% improves the physical properties of chromium-molybdenum steels of low carbon content.

From the above data it will be evident that I have made an important contribution to the art of metallurgy by the provision of a steel of superior weldability and with physical properties in excess of the requirements for steels of this type in commercial practice. 10

It should be understood that the invention is not limited to the particular examples which have been given for purposes of illustration, but may be otherwise embodied within the scope of the following claims: 15

I claim:

1. A cast steel article composed of: 2 to 10 per cent chromium, 0.5 to 2.0 per cent molybdenum, usual amounts of silicon, manganese, sulphur and phosphorus, containing at least 0.75 per cent but not over 1.5 per cent nickel, not over 0.10 per cent carbon, and the balance iron and incidental impurities characterized by improved strength and welding characteristics. 20

2. A welded construction made of cast steel of the following composition: 2 to 10 per cent chromium, 0.5 to 2.0 per cent molybdenum, usual amounts of silicon, manganese, sulphur and phosphorus, containing at least 0.75 per cent but not over 1.5 per cent nickel, not over 0.10 per cent carbon, and the balance iron and incidental impurities.

NICHOLAS A. ZIEGLER.

#### REFERENCES CITED

The following references are of record in the file of this patent:

#### UNITED STATES PATENTS

| Number    | Name         | Date          |
|-----------|--------------|---------------|
| 882,112   | Illingworth  | Mar. 17, 1908 |
| 2,059,746 | Ritterhausen | Nov. 3, 1936  |
| 2,227,891 | Rose         | Jan. 7, 1941  |
| 2,281,219 | Ziegler      | Apr. 28, 1942 |

#### OTHER REFERENCES

Alloys of Iron and Chromium, vol. I, Low Chromium, page 467, published in 1937 by the McGraw-Hill Book Co., New York.